

## UNITED STATES PATENT OFFICE

2,243,059

PROCESS FOR THE MANUFACTURE OF  
WORKING PIECES IMPERMEABLE TO GAS  
AND VACUUM PROOF

Hans Bernstorff, Frankfort-on-the-Main, Germany, assignor, by mesne assignments, to Chemical Marketing Company Inc., New York, N. Y.

No Drawing. Application March 10, 1939, Serial No. 261,134. In Germany March 21, 1938

## 3 Claims. (Cl. 148—2)

My invention relates to a process for the manufacture of working pieces which are vacuum proof and impermeable to gas, such as, for instance, sheets, discs, plates and the like, made of beryllium or its alloys with a high content of beryllium.

Owing to the low ductility of beryllium or such alloys which have a high content of beryllium, as for instance, alloys of beryllium and aluminium with for example more than 80 percent of beryllium, it has proved very difficult to manufacture therefrom working pieces such as sheets, discs or the like which moreover are also impermeable to gas and vacuum proof.

Now I have found that according to my invention working pieces such as sheets, discs and the like which meet these requirements may be manufactured by casting an ingot of the metal or the alloy, whereby the casting or the ingot is free of occlusions, pores and shrinkholes and then dividing this solid ingot or casting by sawing, cutting, milling or the like into suitable sheets, discs or the like, such an ingot or casting of beryllium or its alloys which is free of shrinkholes and impermeable may be made, for instance, by melting down the metal under high vacuum, for example, under pressures below .01 mm. of mercury, and heating the melt for a period of time such as, for example, for one-half hour to one hour, to a temperature which is about 100° C. and more above the fusion point thereof, and then cooling down the melted product under high vacuum.

According to my invention these sheets, discs and the like may be subjected to a further treatment, if for instance instead of plain and flat working pieces a curved surface is desired. In the latter case it has been proved advantageous to heat the working pieces in a protecting atmosphere, for instance, hydrogen, to temperatures below the fusion point of beryllium or the alloy and then forming the working pieces with pressure in a suitable manner. Furthermore it has been found that it is advantageous to work at temperatures which lie about 50 to 100° centigrade below the fusion point of the working substance. The pressures which are necessary for the treatment depend mostly on the used temperature and may easily be determined by experiments.

Sheets, discs and so on which are made according to my invention are vacuum proof and even impermeable against high vacuum. They may be utilized, for instance, as windows for the emission of rays from X-ray tubes. If desired, the working pieces may also be subjected to a

further treatment or improvement by polishing, coating with electrodeposited coatings or the like.

What I claim is:

1. A process for the manufacture of occlusion-free articles of a material selected from the group consisting of beryllium and beryllium alloys having a high content of beryllium, such as sheets, plates and discs, which are impermeable to gas and vacuum-proof, comprising heating a batch of such material under high vacuum to a temperature substantially above the melting point thereof for at least one-half an hour, then allowing the melted batch to cool under high vacuum to form an ingot, dividing this ingot into work pieces of the type of sheets and discs, and then heating such work pieces to temperatures between 50° C. and 100° C. below the melting point thereof under a protecting atmosphere and forming such heated work pieces under pressure.
2. A process for the manufacture of occlusion-free articles of a material selected from the group consisting of beryllium and beryllium alloys having a high content of beryllium, such as, sheets, plates and discs, which are impermeable to gas and vacuum-proof, comprising heating a batch of such material under high vacuum to a temperature at least about 100° C. over the melting point thereof for at least one-half an hour, then allowing the melted batch to cool under high vacuum to form an ingot, dividing this ingot into work pieces of the type of sheets and discs, and then heating such work pieces to temperatures between 50° C. and 100° C. below the melting point thereof under a protecting atmosphere and forming such heated work pieces under pressure.
3. A process for the manufacture of occlusion-free articles of an alloy of beryllium and aluminum containing more than 80% of beryllium which are impermeable to gases and vacuum-proof, comprising heating a batch of such alloy under high vacuum to a temperature substantially above the melting point thereof for at least one-half an hour, then allowing the melted batch to cool under high vacuum to form an ingot, dividing this ingot into work pieces of the type of sheets and discs, and then heating such work pieces to temperatures between 50° C. and 100° C. below the melting point thereof under a protecting atmosphere and forming such heated work pieces under pressure.

HANS BERNSTORFF.